

No. 776,158.

PATENTED NOV. 29, 1904.

R. A. B. WALSH.

METHOD OF MAKING WIRED GLASS.

APPLICATION FILED FEB. 8, 1904.

NO MODEL.

*Fig. 1.*



*Fig. 2.*



*Fig. 3.*



*Fig. 4.*



Witnesses:

G. A. Pennington  
J. H. Miskrood

Inventor:  
Robert A. B. Walsh,  
by Bakewell Cornwall  
Atty's.

## UNITED STATES PATENT OFFICE.

ROBERT A. B. WALSH, OF ST. LOUIS, MISSOURI, ASSIGNOR TO MISSISSIPPI GLASS COMPANY, OF ST. LOUIS, MISSOURI, A CORPORATION OF MISSOURI.

## METHOD OF MAKING WIRED GLASS.

SPECIFICATION forming part of Letters Patent No. 776,158, dated November 29, 1904.

Application filed February 8, 1904. Serial No. 192,506. (No model.)

*To all whom it may concern:*

Be it known that I, ROBERT A. B. WALSH, a citizen of the United States, residing at the city of St. Louis, State of Missouri, have invented a certain new and useful Improvement in Methods of Making Wired Glass, of which the following is a full, clear, and exact description, such as will enable others skilled in the art to which it appertains to make and use the same, reference being had to the accompanying drawings, forming part of this specification, in which—

Figure 1 is a diagrammatical view of the mechanism for forming the glass into sheets with a filler of mesh, the mesh and glass being illustrated in their correlated positions. Fig. 2 is a fragmentary plan view of the two feed-rolls. Fig. 3 is a diagrammatical view of a slightly-modified form of feed mechanism and pressing device, and Fig. 4 is a fragmentary plan view of the feed-rolls and the presser-roll.

This invention relates to a new and useful method of making wired glass, being particularly applicable to rolled glass which is configured with designs or provided with prismatic ribs. Heretofore in the manufacture of the wired glass machines have been employed for embedding the wire mesh in the sheet of glass, and these machines have been of various types. The principal machines, however, resorted to an advance smooth roller which initially rolled the glass into sheet form, a corrugated roller embedding the wire mesh in the center of the sheet, the sheet being finished by a smooth following roller which closed up the openings resulting from the corrugated roller and the embedded wire mesh.

Attempts have been made to configure one surface of wired glass, and as two principal methods have been followed in configuring glass these have been tried in conjunction with the wired glass. These methods involve, first, a configured following roller which impressed its design on the upper surface of the sheet of glass when in a molten or semimolten state and, second, configuring the bed-plate with the design and spreading the glass over such

configured surface. In some instances where it has been desired to configure both surfaces 50 the following roller and configured bed-plate have been conjointly used.

The difficulties attending the practice of configuring the upper surface of a sheet of glass either by a design or prismatic ribs have 55 been caused principally on account of the difference in circumferential speed with respect to the projections of the design on the roller as compared to the grooves of the design on the roller, the difference in circumferential 60 speed causing the glass to crack and check. The difficulty in impressing a design on the bottom of the sheet has been caused principally by the hot molten glass filling the configurations of the table-bed, which has a chilling effect thereon, with the result that the projections become congealed and contracting 65 disproportionately to the body of the sheet will crack or check.

According to my present invention I first 70 form the molten glass into a sheet and by the use of a corrugated roller embed the wire mesh in the center of the sheet, after which one surface, preferably the under surface, is exposed to atmosphere, so as to become slightly 75 cooler than the other surface of the sheet, this cooler surface being then pressed on the configured surface to partake of the design engraved thereon. So far as I am aware I am the first to introduce wire mesh into a sheet 80 of glass from the under side, permit the under side to become slightly cool, and then close the openings and impress a design on the cooled under side by pressure exerted from above. 85

In the accompanying drawings I have shown two forms of apparatus for carrying out my invention, one involving movable rollers and a stationary bed-plate and the other stationarily-mounted rollers and a movable bed-plate. 90

Referring to Fig. 1, 1 is a smooth roller, and 2 a corrugated roller, which are spaced apart to initially form a sheet of glass. The corrugations of roller 2 become impressed in the design so as to locate the wire mesh 3 in the center of the sheet. Means are provided for caus-

ing the travel of these rollers along the bed-  
plate 4, the upper surface of which is con-  
figured, provided with surfaces for imparting  
prismatic ribs to the sheet of glass. In oper-  
5 ation the batch of glass is placed above and be-  
tween the rollers and the wire mesh is prefer-  
ably fed over the corrugated roller 2. These  
rollers 1 and 2 being rotated in the direction  
10 of the arrows they will initially form the sheet  
of glass with the wire mesh embedded in the  
center thereof, said sheet of glass following  
the roller 1, its lower or cooler surface contact-  
ing with the configured bed-plate, the roller  
1 pressing the same against said bed-plate,  
15 so as to impress the configurations thereof  
onto the lower surface of said sheet. In this  
way the cooled lower surface will partake of  
the design; but by reason of the fact that it  
has already been chilled it will not contract  
20 disproportionately or to such an extent that  
it will check or crack with respect to the body  
of the sheet.

In Fig. 3 I have shown the same apparatus  
with this exception, that instead of the roller  
25 1 being used to press the sheet onto the con-  
figured table an independently-mounted roller  
6 is employed for this purpose. In this way  
both surfaces of the sheet of glass are exposed  
30 to atmosphere before the glass is deposited on  
the table, the table being movable with respect  
to the rollers in this form in a well-known  
manner.

I am aware that changes may be made in the  
construction and arrangement of the appara-  
35 tus for carrying out my invention, and there-  
fore I do not wish to be understood as limiting  
myself to the forms shown.

Having thus described the invention, what  
is claimed as new, and desired to be secured by  
Letters Patent, is—

1. The herein-described method of making  
configured wired glass, which consists in em-  
bedding a wire mesh in molten glass, forming  
the same in a sheet, exposing the under side of  
45 the sheet for a brief period to atmosphere for  
the purpose of slightly cooling the same and  
then pressing the under surface of the sheet  
against a configured surface; substantially as  
described.

2. The herein-described method of making  
50 configured wired glass, which consists in ap-  
plying glass to both sides of a wire mesh, roll-  
ing the same into sheets so that the mesh will  
be enveloped except at the edges of the sheet,  
then briefly exposing the glass sheet to atmos-  
55 phere and finally pressing the sheet against a  
configured surface; substantially as described.

3. The herein-described method of making  
wired glass which consists in forcing a wire  
mesh into molten glass and permitting the  
60 glass to flow through the mesh so as to center  
the glass therein by forming the same in a  
sheet, exposing the under side of the sheet for  
a brief period to atmosphere for the purpose  
of slightly cooling the same, and then pressing  
65 the under surface of the sheet against a bed or  
table; substantially as described.

In testimony whereof I hereunto affix my  
signature, in the presence of two witnesses, this  
5th day of February, 1904.

ROBERT A. B. WALSH.

Witnesses:

B. F. FUNK,  
GEORGE BAKEWELL.